

## UNITED STATES PATENT OFFICE

BROR CHRISTIANSEN, OF SMEDJEBACKEN, SWEDEN

## METHOD OF AGGLOMERATING PULVERULENT ORES

No Drawing. Application filed October 30, 1928, Serial No. 316,113, and in Sweden November 8, 1927.

In agglomerating pulverulent iron ores, by sintering or briquetting it has been established that pulverulent magnetites almost without exception are easy to sinter or briquette while pulverulent hematites often cannot be agglomerated in this way. Also in the case that the sintering or briquetting of pulverulent hematite ores really succeeded the resulting product, as a rule, had a very low mechanical resistance. It has been tried to obtain a satisfactory result by admixing to the hematite ore, pulverulent magnetite or other materials, preferably limestone or quartz. It has also been proposed to reduce the hematite to magnetite before sintering it. The low or totally absent power of agglomeration in pulverulent hematite in comparison with pulverulent magnetite has not previously been indisputably explained.

My experiments have shown that pulverulent hematite which cannot be sintered or briquetted in the usual well-known manner owing to their defective power of agglomeration can be well agglomerated if the ore is first finely crushed to a flour-like product corresponding to a grain size of 0.04 millimeters or less. However, the ore shall not be crushed to a colloidal or slimy consistency. The defective power of agglomeration of pulverulent hematites, as a matter of fact, in the first place seems to depend upon the failing adhesive power of the greater grains of the pulverulent ore. But if the ore is sufficiently finely ground the grains of the pulverulent ore obtain such adhesive power also in dry state and sinter together without difficulty, when heated.

The principle of my invention is, therefore, that in agglomerating pulverulent hematites which could not hitherto be suitably agglomerated by sintering, briquetting or any other way the grains of the ore are rendered adhesive to each other by being subjected to a fine-crushing carried very far but not to the colloidal state and thereafter the agglomeration is carried out without difficulty.

My invention is applicable to all known methods of agglomerating pulverulent ores by heating and to all such methods combined with a reduction of the ore, such as the method

of pressing briquettes which are sintered by heating, the agglomeration in sintering pans by combusting fuel admixed to the ore etc.

In carrying out my method practically it is not necessary to crush all of the pulverulent ore to the fineness of flour. It is sufficient to give such fineness only to such a great portion thereof that the product in its entirety has an adhesion corresponding approximately to that generally characteristic of flour-like products.

What I claim is:—

1. A method of agglomerating pulverulent hematites, comprising crushing the pulverulent ore to such fineness that the main portion of the mass has a grain size of 0.04 millimeters or less but not a colloidal or slimy consistency, and then heating the ore thus crushed.

2. A method of agglomerating pulverulent hematites, comprising crushing the pulverulent ore to such fineness that the main portion of the mass has a grain size of 0.04 millimeters or less but not a colloidal or slimy consistency, forming the ore thus crushed to blocks, and then sintering said blocks.

In testimony whereof I have signed my name.

BROR CHRISTIANSEN.

55

60

65

70

75

80

85

90

95

100